# EUROPEAN PATENT SPECIFICATION

(11) **EP 2 718 479 B1**
(45) Date of publication and mention of the grant of the patent: **14.03.2018**
(21) Application number: 12725321.9
(22) Date of filing: 01.06.2012
(51) Int. Cl.: C23C 22/02, C23C 22/34, C23C 22/44, C23C 22/73, C23C 22/74, C23C 22/76, C23C 22/83, B05D 7/14, B65D 85/804, C09D 5/08, B65D 77/20

(54) **METHOD OF PRODUCING AN ALUMINUM OR ALUMINUM ALLOY STRIP WITH A HEAT-SEAL LACQUER ON A FIRST SURFACE AND AN EPOXIDE BASED STOVE LACQUER ON THE SECOND SURFACE PREVIOUSLY COATED WITH A CHROMIUM-FREE CONVERSION COATING**
VERFAHREN ZUR HERSTELLUNG EINES ALUMINIUM- ODER ALUMINIUMLEGIERUNGSSTREIFENS MIT EINER WÄRMEVERSIEGELUNGSLACKIERUNG AUF EINER ERSTEN OBERFLÄCHE UND EINER EPOXIDBASIERTEN EINBRENNLACKIERUNG AUF DER ZWEITEN, ZUVOR MIT EINER CHROMFREIEN KONVERSIONSBESCHICHTUNG BESCHICHTETEN OBERFLÄCHE
PROCÉDÉ DE PRODUCTION D'UNE BANDE D'ALUMINIUM OU D'ALLIAGE D'ALUMINIUM DOTÉE D'UNE LAQUE DE THERMOSCELLAGE SUR UNE PREMIÈRE SURFACE ET D'UNE LAQUE CUITE AU FOUR À BASE D'ÉPOXYDE SUR LA SECONDE SURFACE PRÉALABLEMENT REVÊTUE D'UNE COUCHE DE CONVERSION EXEMPTE DE CHROME

(30) Priority: 10.06.2011 EP 11004742
(43) Date of publication of application: 16.04.2014
(73) Proprietor: Amcor Flexibles Kreuzlingen Ltd., 8280 Kreuzlingen (CH)
(72) Inventor: LUTZ, Jürg, CH-9404 Rorschacherberg (CH); SEGERER, René, CH-9100 Herisau (CH); SCHLAGER, Hans, CH-9030 Abtwil SG (CH)
(74) Representative: Gernet, Samuel Andreas
(86) International application number: PCT/EP2012/002324
(87) International publication number: WO 2012/167889

(56) References cited:
- EP-A1- 1 859 926
- EP-A1- 2 048 203
- US-A1- 2004 062 873
- US-A1- 2009 214 883
- US-A1- 2010 055 327
- US-B1- 6 346 295

## Description

The invention relates to a method of producing an aluminium or aluminium alloy strip with a heat-seal lacquer on a first surface and an epoxide based stove lacquer on the second surface.

In particular, the invention relates to the preparation of cleaned surfaces with good adhesion properties of the aforementioned organic coatings on aluminium or aluminium alloy strips intended for the manufacturing of lacquered and deep-drawn capsules closed with a heat-sealed membrane lid for packaging portions of coffee.

So-called "rinse" and "no-rinse" processes are generally known in the chemical treatment of metal surfaces, for example for the subsequent application of paints, adhesives and/or plastics. In rinse and no-rinse processes, the metal surfaces are freed from oil, dirt and other residues in a first stage. Any residues of chemicals from this first stage are removed by rinsing with water. In the next stage of the rinse process, the clean metal surface is wetted with an aqueous bath solution which is rinsed off. In the non-rinse process the clean metal surface is wetted with an aqueous bath solution which is not rinsed off, but instead is dried in situ on the metal surface and, in the process, is converted into a solid film of the bath ingredients. Coatings such as these can significantly improve the surface quality of covering layers subsequently applied, particularly with respect to corrosion control and adhesion. Originally, treatment solutions containing hexavalent chromium ("yellow chromating") were often proposed in the extensive relevant prior art literature. On account of the toxic character of Cr(VI), these processes or rather the rinsing waters accumulating therein require expensive wastewater treatment. Even processes which only use trivalent chromium were not entirely satisfactory on account of increasing demands for the complete absence of chromium.

The chromium-free conversion treatment of aluminum surfaces with fluorides of boron, silicon, titanium zirconium or molybdenum alone or in conjunction with organic polymers for obtaining permanent protection against corrosion and for producing a base for subsequent painting is known in principle:
US-A-5,129,967 and US-A-4,921,552 disclose treatment baths for the no-rinse treatment (described there as "dried in place conversion coating") of aluminum containing:
   a) 10 to 16 g/l of polyacrylic acid or homopolymers thereof,
   b) 12 to 19 g/l of hexafluoro zirconic acid,
   c) 0.17 to 0.3 g/l of hydrofluoric acid and
   d) up to 0.6 g/l of hexafluoro titanic acid.
EP-A-0 008 942 discloses treatment solutions, preferably for aluminum cans, containing:
   a) 0.5 to 10 g/l of polyacrylic acid or an ester thereof and
   b) 0.2 to 8 g/l of at least one of the compounds H₂ ZrF₆, H₂TiF₆ and H₂SiF₆, the pH value of the solution being below 3.5, and an aqueous concentrate for regenerating the treatment solution containing:
      a) 25 to 100 g/l of polyacrylic acid or an ester thereof,
      b) 25 to 100 g/l of at least one of the compounds H₂ ZrF₆, H₂TiF₆ and H₂SiF₆ and
      c) a source of free fluoride ions supplying 17 to 120 g/l of free fluoride.
DE-C-24 33 704 describes treatment baths for increasing paint adhesion and permanent protection against corrosion inter alia on aluminum which may contain from 0.1 to 5 g/l of polyacrylic acid or salts or esters thereof and 0.1 to 3.5 g/l of ammonium fluorozirconate, expressed as ZrO₂.
US-A-4,992,116 describes treatment baths for the conversion treatment of aluminum with pH values of around 2.5 to 5 which contain at least three components, namely:
   a) phosphate ions in a concentration of 1.1x10⁻⁵ to 5.3x10⁻³ moles/I, corresponding to 1 to 500 mg/l,
   b) 1.1 x 10⁻⁵ to 1.3 x 10⁻³ moles/l of a fluoroacid of an element of the group consisting of Zr, Ti, Hf and Si (corresponding to 1.6 to 380 mg/l, depending on the element) and
   c) 0.26 to 20 g/l of a polyphenol compound obtainable by reacting poly(vinylphenol) with aldehydes and organic amines.

WO-A-92/07973 describes a chromium-free treatment process for aluminum which uses 0.01 to around 18% by weight of H₂ZrF₆ and 0.01 to around 10% by weight of a 3-(N-C₁₋₄-alkyl-N-2-hydroxyethylaminomethyl)-4-hydroxystyrene polymer as essential components in the form of an acidic aqueous solution.

DE-A-43 17 217 describes a process for the pretreatment of surfaces of aluminum or its alloys before a second conversion treatment for permanent corrosion control, in which the surfaces are contacted with acidic aqueous treatment solutions which contain complex fluorides of the elements boron, silicon, titanium, zirconium or hafnium either individually or in admixture with one another in concentrations of the fluoroanions of, in total, 100 to 4,000 and preferably 200 to 2,000 mg/l and which have a pH value of 0.3 to 3.5 and preferably in the range from 1 to 3. The treatment solutions may additionally contain polymers of the polyacrylate type and/or in the form of reaction products of poly(vinylphenol) with aldehydes and organic hydroxyfunctional amines in concentrations below 500 mg/l and preferably below 200 mg/l. Phosphoric acid is another optional constituent of these baths.

US-A-4,136,073 claims a chromium-free treatment process for aluminum surfaces, in which the surfaces are contacted with acidic (pH 1.2 to 5.5) aqueous solutions containing an organic film former and a soluble titanium compound in a ratio by weight of polymer to titanium of 100:1 to 1 :10. The preferred titanium concentration is between 0.01 and 5% by weight.

US-A-5,868872 discloses a chromium-free process for the no-rinse treatment of aluminium and its alloys and aqueous bath solutions suitable for this process. The surfaces are contacted with solutions containing:
a) 2.2 to 22.0 g/l of Zr(IV) and/or 1.4 to 14.0 g/l of Ti(IV),
b) 2.4 to 24.0 g/l of orthophosphate,
c) 3.0 to 30.0 g/l of fluoride,
d) 0.15 to 1.5 g/l of a water-soluble or homogeneously water-dispersible organic film former, and the solutions are dried on the surface without rinsing after a contact time of 1 to 40 seconds at temperatures of 50°C to 125°C.
US6346295 B1 discloses a method for coating an aluminum or aluminum alloy strip in a continuous production line with a Cr-free conversion coating solution comprising complex fluorides of titanium and /or zirconium.
US 2009214883 A1 discloses a method of producing a Cr-free conversion coating on aluminum or aluminum alloy strip by treating with a solution comprising H₂TiF₆ or H₂ZrF₆ and ammonium molybdate.
EP2048203 A1, US2004062873A describe a method of producing a Cr-free conversion coating on an aluminum or aluminum alloy strip with a silane-containing solution. An object of the present invention is to provide a method as defined in claim 1 with a good adhesion of the aluminium or aluminium alloy strip with a heat-seal lacquer on a first surface and an epoxide based stove lacquer on the second surface and the epoxide based stove lacquer without the need of a Cr(III) conversion coating. In particular, the aluminium or aluminium alloy strip manufactured with the method according to the present invention shall be qualified for the manufacture of deep-drawn capsules for packaging portions of coffee, the capsules having a heat-seal lacquer on the inner surface of the capsule and an epoxide based coloured stove lacquer on the outer surface of the capsule. The method includes the step of producing a chromium-free conversion coating on a surface of an aluminium or aluminium alloy strip in a continuous production line, the chromium-free conversion coating having good adhesion properties of a heat-seal lacquer on a first surface and an epoxide based stove lacquer on the second surface of the aluminium or aluminium alloy strip intended for the manufacturing of lacquered and deep-drawn capsules closed with a heat-sealed membrane lid for packaging portions of coffee.

The aforementioned objective is achieved by way of the invention in that a chromium-free conversion coating is produced on the first and second surface of the aluminium or aluminium alloy strip in a continuous production line before applying the heat-seal lacquer and the stove lacquer, the chromium-free conversion coating is produced by
(A) a no-rinse process by treatment with a solution of silanes in a polar organic solvent, or
   a no-rinse process by treatment with an aqueous solution of 5 to 10 wt.-% hexafluorotitanic acid (H₂TiF₆) and 2.5 to 5 wt.-% hexafluorozirconic acid (H₂ZrF₆), or
(B) a rinse process by treatment with an aqueous solution of < 1 wt.-% diammonium dimolybdate ((NH₄)₂Mo₂O₇) and 5 to 10 wt.-% hexafluorozirconic acid (H₂ZrF₆).
The method of producing a chromium-free conversion coating on a surface of an aluminum or aluminum alloy strip in a continuous production line as defined in claim 1 comprises the steps of continuous uncoiling of a rolled aluminium or aluminium alloy strip from a first coil;
continuous annealing of the uncoiled strip;
continuous cleaning and degreasing of the surface of the annealed strip;
continuous washing of the cleaned and degreased surface of the strip;
continuous pickling of the surface of the washed strip;
continuous washing of the surface of the pickled strip;
drying of the surface of the washed strip;
continuous production of a chromium-free conversion coating on the surface of the dried conversion coated strip by
(A) a no-rinse process by treatment with a solution of silanes in a polar organic solvent, or
   a no-rinse process by treatment with an aqueous solution of 5 to 10 wt.-% hexafluorotitanic acid (H₂TiF₆) and 2.5 to 5 wt.-%hexafluorozirconic acid (H₂ZrF₆), or
(B) a rinse process by treatment with an aqueous solution of < 1 wt.-% diammonium dimolybdate ((NH₄)₂Mo₂O₇) and 5 to 10 wt.-% hexafluorozirconic acid (H₂ZrF₆);
optional washing of the surface of the conversion coated strip;
continuous drying of the surface of the conversion coated and optionally washed strip;
continuous coiling of the dried strip onto a second coil.

Cleaning and degreasing is preferably made by spraying the strip with an aqueous solution of 5 to 50 g/l, preferably 15 to 25 g/l, of an initial solution comprising 0.10 to 1.0 wt.-% bisoctyl dimethyl ammonium chloride, 5 to 10 wt.-% potassium hydroxide, 5 to 10 wt.-% phosphate (P) and < 5 wt.-% cationic tenside.

In a first embodiment of the invention, pickling is preferably made by spraying the strip with an aqueous solution of 5 to 50 g/l, preferably 15 to 25 g/l, of an initial solution comprising 65 to 80 wt.-% ortho phosphoric acid.

In a second embodiment of the invention, pickling is preferably made by spraying the strip with an aqueous solution of 5 to 30 g/l, preferably 8 to 15 g/l, of a first initial solution comprising 25 to 50 wt.-% sulphuric acid and 5 to 15 wt.-% non ionic tenside, and 0.1 to 10 g/l, preferably 1 to 3 g/l, of a second initial solution comprising 5 to 7 wt.-% hydrofluoric acid.

In a first embodiment of the invention, the conversion coating is preferably made by spraying the strip with a solution of 50 to 200 g/l, preferably 80 to 120 g/l, of an initial solution comprising silane and 10 to 25 wt.-% ethanol.

In a second embodiment of the invention, the conversion coating is preferably made by spraying the strip with an aqueous solution of 10 to 160 g/l, preferably 30 to 50 g/l, of a first initial solution comprising 5 to 10 wt.-% hexafluorotitanic acid and 2.5 to 5 wt.-% hexafluorozirconic acid, and 1 to 10 g/l, preferably 7 to 9 g/l, of a second initial solution comprising 20 to 21 wt.-% silica.

In a third embodiment of the invention, the conversion coating is preferably made by spraying the strip with an aqueous solution of 5 to 50 g/l, preferably 15 to 25 g/l, of a first initial solution comprising < 1 wt.-% diammonium dimolybdate and 5 to 10 wt.-% hexafluorozirconic acid, and 0.01 to 0.3 g/l, preferably 0.1 to 0.3 g/l, of a second initial solution comprising 10 to 25 wt.-% ammonium fluoride and 10 to 25 wt.-% ammonium hydrogen difluoride.

In a third embodiment of the invention, the conversion coating is preferably made by spraying the strip with an aqueous solution of 5 to 50 g/l, preferably 15 to 25 g/l, of a first initial solution comprising < 1 wt.-% diammonium dimolybdate and 5 to 10 wt.-% hexafluorozirconic acid, and 0.01 to 0.3 g/l, preferably 0.1 to 0.3 g/l, of a second initial solution comprising 10 to 25 wt.-% ammonium fluoride and 10 to 25 wt.-% ammonium hydrogen difluoride, and 0 to 2 g/l, preferably 0.05 to 0.2 g/l, of a third initial solution comprising 25 wt.-% polycarboxylic acid in water.

In the preferred no rinse process according to the invention, a conventionally cleaned and rinsed metal surface, after rinsing with deionized water and drying and/or removal of the water film by squeegees, is wetted in any manner with the solution of silanes in the polar organic solvent aqueous treatment solution in such a quantity that around 2 to 20 ml and preferably around 5 to 10 ml of the polar organic treatment solution are applied per square meter of surface area.

The treatment solutions in the preferred no rinse process according to the invention may be applied to the precleaned metal strips by any method which is capable of producing a uniform, defined liquid film on the metal surface in the quantity ranges indicated. The roller application process using two to four rollers ("chemcoater") has proved to be particularly effective, although wetting of the strip by spraying or immersion and subsequent removal of the excess liquid film, for example by plastic-coated equalizing rollers or an adjustable air knife, is also suitable. The temperature of the treatment solution may be in the range from 15°C to 30°C and is preferably in the range from 20°C to 25°C. The liquid film applied to the metal surface is allowed to react thereon for about 1 to 40 seconds, after which the film is dried and heat-treated at elevated temperature. However, the process steps of contact with the metal surface and drying may also be combined. After drying, a formable, water-insoluble solid film with a weight per unit area of around 5 to 50 mg Si/m² and preferably around 10 to 30 mg Si/m² is left on the metal surface. The drying and/or heat treatment of the liquid film applied to the metal surface, or rather of the chemicals applied with it, may be carried out at temperatures of around 80°C to 140°C, temperatures in the range from 110°C to 120°C being preferred.

Both acidic and alkaline cleaners are suitable for the cleaning pretreatment of the aluminum surfaces to be wetted in accordance with the invention. The layers obtained with the treatment solution according to the invention provide a uniform finish of the aluminum substrate. In combination with the organic coatings subsequently applied, they satisfy the requirements of the food packaging industry.

The following example relates to a no-rinse process with a conversion coating by treatment with a solution of silanes in ethanol.
1. cleaning and degreasing with surfactant-containing alkaline or acidic cleaners -- for example GARDOCLEAN S 5664, 20 g/l -- applied by spraying at a treatment temperature of 50°C to 65°C for treatment times of 2 to 5 s,
2. rinsing with process water,
3. pickling with an aqueous solution of 20 g/l phosphoric acid (H₃PO₄) or 10.6 g/l sulfuric acid (H₂SO₄ with 2 g/l hydrofluoric acid (HF) applied by spraying at a treatment temperature of 50°C to 60°C for treatment times of 2 to 5 s,
4. rinsing with deionized water,
5. drying,
6. application of the pretreatment -- for example 100g/l OXSILAN® MM-0705using a coater at a treatment temperature of 18°C to 25°C, 20 mg Si/m²
7. drying (with OXSILAN® at 110°C to 120°C)

Chemical composition, broad and preferred of treatment solutions for the process steps of degreasing, pickling and conversion related to rinse and no rinse processes are included in the following tables.

**Table 1: No rinse process, conversion with silanes**

| **Process step** | **Initial Solution** | **Bath concentration [g/l]** | |
|---|---|---|---|
| | | **broad range** | **preferred range** |
| Degreasing (spraying) | Gardoclean S 5664 | 5-50 | 15-25 |
| Pickling 1 (spraying) | Gardobond H 7173 | 5-50 | 15-25 |
| Pickling 2 (spraying) | Gardoclean S 5240/2 | 5-30 | 8-15 |
| | Gardobond H 7269 | 0.1-10 | 1-3 |
| Conversion (no rinse) | Oxsilan MM-0705 | 50-200 | 80-120 |

**Table 2: No rinse process, conversion with Zr/Ti**

| **Process step** | **Initial Solution** | **Bath concentration [g/l]** | |
|---|---|---|---|
| | | **broad range** | **preferred range** |
| Degreasing (spraying) | Gardoclean S 5664 | 5-50 | 15-25 |
| Pickling 1 (spraying) | Gardobond H 7173 | 5-50 | 15-25 |
| Pickling 2 (spraying) | Gardoclean S 5240/2 | 5-30 | 8-15 |
| | Gardobond H 7269 | 0.1-10 | 1-3 |
| Conversion (no rinse) | Gardobond X 4591 | 10-160 | 30-50 |
| | GTB 10437B (Additive) | 1-10 | 7-9 |

**Table 3: Rinse process, conversion with Zr/Mo**

| **Process step** | **Initial Solution** | **Bath concentration [g/l]** | |
|---|---|---|---|
| | | **broad range** | **preferred range** |
| Degreasing (spraying) | Gardoclean S 5664 | 5-50 | 15-25 |
| Pickling (spraying) | Gardobond H 7173 | 5-50 | 15-25 |
| Conversion 1 (rinse) | Permatreat 1903 A | 5-50 | 30-50 |
| | Gardobond H 7255 | 0.01-0.3 | 0.1-0.3 |
| Conversion 2 (rinse) | Permatreat 1903 A | 5-50 | 15-25 |
| | Gardobond H 7255 | 0.01-0.3 | 0.1-0.3 |
| | Gardolene D 6815 | 0-2 | 0.05-0.2 |

**Table 4: Chemical Composition of the Initial Solutions**

| **Inititial Solution** | **Chemical composition** | **[weight-%]** |
|---|---|---|
| Gardoclean S 5664 | bisoctyl dimethyl ammonium chloride | 0.10-1.0 |
| | potassium hydroxide | 5-10 |
| | phosphate (P) | 5-10 |
| | cationic tenside | < 5 |
| Gardobond H 7173 | ortho phosphoric acid | 65-80 |
| Gardoclean S 5240/2 | sulfuric acid | 25-50 |
| | non ionic tenside | 5-15 |
| Gardobond H 7269 | hydrofluoric acid | 5-7 |
| Oxsilan MM-0705 | silane | |
| | ethanol | 10-25 |
| Gardobond X 4591 | hexafluorotitanic acid | 5-10 |
| | hexafluorozirconic acid | 2.5-5 |
| GTB 10437B additive | Silica | 20-21 |
| Permatreat 1903 A | diammonium dimolybdate | <1 |
| | hexafluorozirconic acid | 5-10 |
| Gardobond H 7255 | ammonium fluoride | 10-25 |
| | ammonium hydrogen difluoride | 10-25 |
| Gardolene D 6815 | polycarboxylic acid in water (polymer) | 25 |

## Claims

1. Method of producing an aluminium or aluminium alloy strip with a heat-seal lacquer on a first surface and an epoxide based stove lacquer on the second surface,
**characterised in that**
a chromium-free conversion coating is produced on the first and second surface of the aluminium or aluminium alloy strip in a continuous production line before applying the heat-seal lacquer and the stove lacquer, the chromium-free conversion coating is produced by
(A) a no-rinse process by treatment with a solution of silanes in a polar organic solvent, or
a no-rinse process by treatment with an aqueous solution of 5 to 10 wt.-% hexafluorotitanic acid (H₂TiF₆) and 2.5 to 5 wt.-% hexafluorozirconic acid (H₂ZrF₆), or
(B) a rinse process by treatment with an aqueous solution of < 1 wt.-% diammonium dimolybdate ((NH₄)₂Mo₂O₇) and 5 to 10 wt.-% hexafluorozirconic acid (H₂ZrF₆).

2. Method of producing a chromium-free conversion coating on a surface of an aluminium or aluminium alloy strip in a continuous production line according to claim 1, the method comprising the steps of
continuous uncoiling of a rolled aluminium or aluminium alloy strip from a first coil;
continuous annealing of the uncoiled strip;
continuous cleaning and degreasing of the surface of the annealed strip;
continuous washing of the cleaned and degreased surface of the strip;
continuous pickling of the surface of the washed strip;
continuous washing of the surface of the pickled strip;
drying of the surface of the washed strip;
continuous production of a chromium-free conversion coating on the surface of the dried conversion coated strip;
optional washing of the surface of the conversion coated strip; continuous drying of the surface of the conversion coated and optionally washed strip; continuous coiling of the dried strip onto a second coil.

3. Method according to claim 2, wherein cleaning and degreasing is made by spraying the strip with an aqueous solution of 5 to 50 g/l, preferably 15 to 25 g/l, of an initial solution comprising 0.10 to 1.0 wt.-% bisoctyl dimethyl ammonium chloride, 5 to 10 wt.-% potassium hydroxide, 5 to 10 wt.-% phosphate (P) and < 5 wt.-% cationic tenside.

4. Method according to claim 2, wherein pickling is made by spraying the strip with an aqueous solution of 5 to 50 g/l, preferably 15 to 25 g/l, of an initial solution comprising 65 to 80 wt.-% ortho phosphoric acid.

5. Method according to claim 2, wherein pickling is made by spraying the strip with an aqueous solution of 5 to 30 g/l, preferably 8 to 15 g/l, of a first initial solution comprising 25 to 50 wt.-% sulphuric acid and 5 to 15 wt.-% non ionic tenside, and 0.1 to 10 g/l, preferably 1 to 3 g/l, of a second initial solution comprising 5 to 7 wt.-% hydrofluoric acid.

6. Method according to claim 2, wherein the conversion coating is made by spraying the strip with a solution of 50 to 200 g/l, preferably 80 to 120 g/l, of an initial solution comprising silane and 10 to 25 wt.-% ethanol.

7. Method according to claim 2, wherein the conversion coating is made by spraying the strip with an aqueous solution of 10 to 160 g/l, preferably 30 to 50 g/l, of a first initial solution comprising 5 to 10 wt.-% hexafluorotitanic acid and 2.5 to 5 wt.-% hexafluorozirconic acid, and 1 to 10 g/l, preferably 7 to 9 g/l, of a second initial solution comprising 20 to 21 wt.-% silica.

8. Method according to claim 2, wherein the conversion coating is made by spraying the strip with an aqueous solution of 5 to 50 g/l, preferably 15 to 25 g/l, of a first initial solution comprising < 1 wt.-% diammonium dimolybdate and 5 to 10 wt.-% hexafluorozirconic acid, and 0.01 to 0.3 g/l, preferably 0.1 to 0.3 g/l, of a second initial solution comprising 10 to 25 wt.-% ammonium fluoride and 10 to 25 wt.-% ammonium hydrogen difluoride.

9. Method according to claim 2, wherein the conversion coating is made by spraying the strip with an aqueous solution of 5 to 50 g/l, preferably 15 to 25 g/l, of a first initial solution comprising < 1 wt.-% diammonium dimolybdate and 5 to 10 wt.-% hexafluorozirconic acid, and 0.01 to 0.3 g/l, preferably 0.1 to 0.3 g/l, of a second initial solution comprising 10 to 25 wt.-% ammonium fluoride and 10 to 25 wt.-% ammonium hydrogen difluoride, and 0 to 2 g/l, preferably 0.05 to 0.2 g/l, of a third initial solution comprising 25 wt.-% polycarboxylic acid in water.

## Patentansprüche

1. Verfahren zur Herstellung eines Aluminium- oder Aluminiumlegierungsstreifens mit einem Heißsiegellack auf einer ersten Fläche und einem epoxidbasierten Einbrennlack auf der zweiten Fläche,
**dadurch gekennzeichnet, dass**
eine chromfreie Konversionsbeschichtung auf der ersten und zweiten Fläche des Aluminium- oder Aluminiumlegierungsstreifens in einer kontinuierlichen Produktionsanlage wird, bevor der Heißsiegellack und der Einbrennlack aufgebracht werden, wobei die chromfreie Konversionsbeschichtung hergestellt wird durch
(A) ein No-Rinse-Verfahren durch Behandlung mit einer Lösung von Silanen in einem polaren organischen Lösungsmittel, oder
ein No-Rinse-Verfahren durch Behandlung mit einer wässrigen Lösung von 5 bis 10 Gew.-% Hexafluortitansäure (H₂TiF₆) und 2,5 bis 5 Gew.-% Hexafluorzirkonsäure (H₂ZrF₆), oder
(B) ein Rinse-Verfahren durch Behandlung mit einer wässrigen Lösung von < 1 Gew.-% Diammoniumdimolybdat ((NH₄)₂Mo₂O₇) und 5 bis 10 Gew.-% Hexafluorzirkonsäure (H₂ZrF₆).

2. Verfahren zur Herstellung einer chromfreien Konversionsbeschichtung auf einer Oberfläche eines Aluminium- oder Aluminiumlegierungsstreifens in einer kontinuierlichen Produktionsanlage nach Anspruch 1, wobei das Verfahren die folgenden Schritte umfasst:
kontinuierliches Abrollen eines aufgerollten Aluminium- oder Aluminiumlegierungsstreifens von einer ersten Rolle;
kontinuierliches Glühen des abgerollten Streifens;
kontinuierliches Reinigen und Entfetten der Oberfläche des geglühten Streifens;
kontinuierliches Waschen der gereinigten und entfetteten Oberfläche des Streifens;
kontinuierliches Beizen der Oberfläche des gewaschenen Streifens;
kontinuierliches Waschen der Oberfläche des gebeizten Streifens;
Trocknen der Oberfläche des gewaschenen Streifens;
kontinuierliche Herstellung einer chromfreien Konversionsbeschichtung auf der Oberfläche des getrockneten konversionsbeschichteten Streifens;
optionales Waschen der Oberfläche des konversionsbeschichteten Streifens;
kontinuierliches Trocknen der Oberfläche des konversionsbeschichteten und optional gewaschenen Streifens;
kontinuierliches Aufrollen des getrockneten Streifens auf eine zweite Rolle.

3. Verfahren nach Anspruch 2, wobei das Reinigen und Entfetten durch Besprühen des Streifens mit einer wässrigen Lösung von 5 bis 50 g/l, vorzugsweise 15 bis 25 g/l, einer Ausgangslösung durchgeführt wird, welche 0,10 bis 1,0 Gew.-% Dimethyldioctylammoniumchlorid, 5 bis 10 Gew.-% Kaliumhydroxid, 5 bis 10 Gew.-% Phosphat (P) und < 5 Gew.-% kationisches Tensid umfasst.

4. Verfahren nach Anspruch 2, wobei das Beizen durch Besprühen des Streifens mit einer wässrigen Lösung von 5 bis 50 g/l, vorzugsweise 15 bis 25 g/l, einer Ausgangslösung durchgeführt wird, welche 65 bis 80 Gew.-% Orthophosphorsäure umfasst.

5. Verfahren nach Anspruch 2, wobei das Beizen durch Besprühen des Streifens mit einer wässrigen Lösung von 5 bis 30 g/l, vorzugsweise 8 bis 15 g/l, einer ersten Ausgangslösung, welche 25 bis 50 Gew.-% Schwefelsäure und 5 bis 15 Gew.-% nichtionisches Tensid umfasst, und 0,1 bis 10 g/l, vorzugsweise 1 bis 3 g/l, einer zweiten Ausgangslösung, welche 5 bis 7 Gew.-% Fluorwasserstoffsäure umfasst, durchgeführt wird.

6. Verfahren nach Anspruch 2, wobei die Konversionsbeschichtung durch Besprühen des Streifens mit einer Lösung von 50 bis 200 g/l, vorzugsweise 80 bis 120 g/l, einer Ausgangslösung durchgeführt wird, welche Silan und 10 bis 25 Gew.-% Ethanol umfasst.

7. Verfahren nach Anspruch 2, wobei die Konversionsbeschichtung durch Besprühen des Streifens mit einer wässrigen Lösung von 10 bis 160 g/l, vorzugsweise 30 bis 50 g/l, einer ersten Ausgangslösung, welche 5 bis 10 Gew.-% Hexafluortitansäure und 2,5 bis 5 Gew.-% Hexafluorzirkonsäure umfasst, und 1 bis 10 g/l, vorzugsweise 7 bis 9 g/l, einer zweiten Ausgangslösung, welche 20 bis 21 Gew.-% Siliziumdioxid umfasst, durchgeführt wird.

8. Verfahren nach Anspruch 2, wobei die Konversionsbeschichtung durch Besprühen des Streifens mit einer wässrigen Lösung von 5 bis 50 g/l, vorzugsweise 15 bis 25 g/l, einer ersten Ausgangslösung, welche < 1 Gew.-% Diammoniumdimolybdat und 5 bis 10 Gew.-% Hexafluorzirkonsäure umfasst, und 0,01 bis 0,3 g/l, vorzugsweise 0,1 bis 0,3 g/l, einer zweiten Ausgangslösung, welche 10 bis 25 Gew.-% Ammoniumfluorid und 10 bis 25 Gew.-% Ammoniumhydrogendifluorid umfasst, durchgeführt wird.

9. Verfahren nach Anspruch 2, wobei die Konversionsbeschichtung durch Besprühen des Streifens mit einer wässrigen Lösung von 5 bis 50 g/l, vorzugsweise 15 bis 25 g/l, einer ersten Ausgangslösung, welche < 1 Gew.-% Diammoniumdimolybdat und 5 bis 10 Gew.-% Hexafluorzirkonsäure umfasst, und 0,01 bis 0,3 g/l, vorzugsweise 0,1 bis 0,3 g/l, einer zweiten Ausgangslösung, welche 10 bis 25 Gew.-% Ammoniumfluorid und 10 bis 25 Gew.-% Ammoniumhydrogendifluorid umfasst, und 0 bis 2 g/l, vorzugsweise 0,05 bis 0,2 g/l, einer dritten Ausgangslösung, welche 25 Gew.-% Polycarboxylsäure in Wasser umfasst, durchgeführt wird.

## Revendications

1. Procédé de production d'une bande en aluminium ou en alliage d'aluminium avec une laque de thermoscellage sur une première surface et une laque cuite au four à base d'époxyde sur la deuxième surface,
**caractérisé en ce que**
un revêtement de conversion exempt de chrome est produite sur les première et deuxième surfaces de la bande en aluminium ou en alliage d'aluminium dans une ligne de production en continu avant l'application de la laque de thermoscellage et de la laque cuite au four, le revêtement de conversion exempt de chrome étant produit par
(A) un procédé sans rinçage par traitement avec une solution de silanes dans un solvant organique polaire, ou
un procédé sans rinçage par traitement avec une solution aqueuse de 5 à 10 % en poids d'acide hexafluorotitanique (H₂TiF₆) et de 2,5 à 5 % en poids d'acide hexafluorozirconique (H₂ZrF₆), ou
(B) un procédé avec rinçage par traitement avec une solution aqueuse de moins de 1 % en poids de dimolybdate de diammonium ((NH₄)₂Mo₂O₇) et de 5 à 10 % en poids d'acide hexafluorozirconique (H₂ZrF₆).

2. Procédé de production d'un revêtement de conversion exempt de chrome sur une surface d'une bande en aluminium ou en alliage d'aluminium dans une ligne de production en continu selon la revendication 1, le procédé comprenant les étapes suivantes :
déroulage en continu d'une bande laminée en aluminium ou en alliage d'aluminium à partir d'une première bobine ;
recuit en continu de la bande déroulée ;
nettoyage et dégraissage en continu de la surface de la bande recuite ;
lavage en continu de la surface nettoyée et dégraissée de la bande ;
décapage en continu de la surface de la bande lavée ;
lavage en continu de la surface de la bande décapée ;
séchage de la surface de la bande lavée ;
production en continu d'un revêtement de conversion exempt de chrome sur la surface de la bande dotée d'un revêtement de conversion séchée ;
éventuellement lavage de la surface de la bande dotée d'un revêtement de conversion ; séchage en continu de la surface de la bande dotée d'un revêtement de conversion et éventuellement lavée ;
enroulement en continu de la bande séchée sur une deuxième bobine.

3. Procédé selon la revendication 2, dans lequel le nettoyage et le dégraissage sont effectués par pulvérisation sur la bande d'une solution aqueuse de 5 à 50 g/l, de préférence de 15 à 25 g/l, d'une solution initiale comprenant 0,10 à 1,0 % en poids de chlorure de bis-octyldiméthylammonium, 5 à 10 % en poids d'hydroxyde de potassium, 5 à 10 % en poids de phosphate (P) et moins de 5 % en poids de tensioactif cationique.

4. Procédé selon la revendication 2, dans lequel le décapage est effectué par pulvérisation sur la bande d'une solution aqueuse de 5 à 50 g/l, de préférence de 15 à 25 g/l, d'une solution initiale comprenant 65 à 80 % en poids d'acide orthophosphorique.

5. Procédé selon la revendication 2, dans lequel le décapage est effectué par pulvérisation sur la bande d'une solution aqueuse de 5 à 30 g/l, de préférence de 8 à 15 g/l, d'une première solution initiale comprenant 25 à 50 % en poids d'acide sulfurique et 5 à 15 % en poids d'un tensioactif non-ionique, et de 0,1 à 10 g/l, de préférence de 1 à 3 g/l, d'une deuxième solution initiale comprenant 5 à 7 % en poids d'acide fluorhydrique.

6. Procédé selon la revendication 2, dans lequel le revêtement de conversion est effectué par pulvérisation sur la bande d'une solution de 50 à 200 g/l, de préférence de 80 à 120 g/l, d'une solution initiale comprenant du silane et 10 à 25 % en poids d'éthanol.

7. Procédé selon la revendication 2, dans lequel le revêtement de conversion est effectué par pulvérisation sur la bande d'une solution aqueuse de 10 à 160 g/l, de préférence de 30 à 50 g/l, d'une première solution initiale comprenant 5 à 10 % en poids d'acide hexafluorotitanique et 2,5 à 5 % en poids d'acide hexafluorozirconique, et de 1 à 10 g/l, de préférence de 7 à 9 g/l, d'une deuxième solution initiale comprenant 20 à 21 % en poids de silice.

8. Procédé selon la revendication 2, dans lequel le revêtement de conversion est effectué par pulvérisation sur la bande d'une solution aqueuse de 5 à 50 g/l, de préférence de 15 à 25 g/l, d'une première solution initiale comprenant moins de 1 % en poids de dimolybdate de diammonium et 5 à 10 % en poids d'acide hexafluorozirconique, et de 0,01 à 0,3 g/l, de préférence de 0,1 à 0,3 g/l, d'une deuxième solution initiale comprenant 10 à 25 % en poids de fluorure d'ammonium et 10 à 25 % en poids d'hydrogénodifluorure d'ammonium.

9. Procédé selon la revendication 2, dans lequel le revêtement de conversion est effectué par pulvérisation sur la bande d'une solution aqueuse de 5 à 50 g/l, de préférence de 15 à 25 g/l, d'une première solution initiale comprenant moins de 1 % en poids de dimolybdate de diammonium et 5 à 10 % en poids d'acide hexafluorozirconique, et de 0,01 à 0,3 g/l, de préférence de 0,1 à 0,3 g/l, d'une deuxième solution initiale comprenant 10 à 25 % en poids de fluorure d'ammonium et 10 à 25 % en poids d'hydrogénodifluorure d'ammonium, et de 0 à 2 g/l, de préférence de 0,05 à 0,2 g/l, d'une troisième solution initiale comprenant 25 % en poids d'acide polycarboxylique dans de l'eau.
